

2,789,069

## METHOD FOR IMPROVING THE MACHINABILITY OF STEEL

Elliot S. Nachtman, Park Forest, Ill., assignor to La Salle Steel Co., Hammond, Ind., a corporation of Delaware

No Drawing. Application September 30, 1954,  
Serial No. 459,527

13 Claims. (Cl. 148—4)

This invention relates to plain carbon and alloy steels and to a method of improving the machinability thereof. It is concerned more particularly with a method of improving the machinability of plain carbon and alloy steels accompanied with improvements also in physical and mechanical properties of the steel.

It is an object of this invention to produce and to provide a method for producing plain carbon and alloy steels in which the machinability is improved by means easily and simply carried out during normal steel making and it is a related object to improve the machinability of steel with improvement also in other physical and mechanical properties of the steel, such as strength, resistance to wear, resistance to corrosion and toughness.

Numerous attempts have been made in the past to improve the machinability of such plain carbon and alloy steels. To the present, lead, selenium, sulphur and bismuth have been found to provide noticeable improvements in the machinability of steel when added to provide certain concentration in the steels but certain undesirable conditions have been associated with their use. For example, improved machinability has been secured by the addition of lead in the manufacture of leaded steels but since lead is insoluble in the steel, it is difficult to achieve the desirable uniform distribution of the lead in the steel. In addition, lead releases toxic fumes under the processing conditions with the result that extensive precautions must be taken in the use thereof.

Similarly the distribution of sulphur in the desired concentration in the steel is also difficult to control and unless combined with manganese in substantial amounts, the sulphur will produce an undesirable condition in the steel during rolling, generally referred to as "hot shortness." Bismuth and selenium have been used on a minor scale in stainless steel for the purpose of improving machinability. However, the additional cost occasioned by the use of such materials in desired amounts is a deterrent to their adoption. In addition, these various elements which have been added to steels to improve machinability in many cases cause an undesirable loss in some of the mechanical and physical properties of the steel.

It has been found in accordance with the invention described and claimed in my copending application Ser. No. 390,739, filed November 16, 1953, that the machinability of plain carbon and alloy steels can be improved materially by the addition of lead and copper in combination in amounts ranging from 0.03 to 0.35 percent by weight copper and 0.03 to 0.5 percent by weight lead. The improvements resulting from the combination of copper and lead in such steels have been found to be enhanced further by the presence of sulphur, phosphorus and manganese.

It has now been found that copper alone can be used effectively in appropriate concentrations, without lead, to improve the machinability of plain carbon and alloy steels. It appears from analysis and observations of results that copper alone functions in a manner substantially

unlike that of lead. Whereas lead is substantially insoluble in steel, copper is soluble in steel, and whereas lead reduces some of the other properties of steel, copper provides additional improvements in the strength, corrosion resistance, and impact strength of plain carbon and alloy steel. Unlike lead, the copper in the desired concentration may be added to steel by normal procedure, requiring no special techniques, with practically 100 percent recovery in the steel and with uniform distribution.

To the best of my knowledge, no one before has introduced copper in plain carbon and alloy steels intentionally for the improvement of machinability and such formulation to modify the chemistry of the steel by the presence of copper to improve machinability is believed to represent a completely new concept in the field of metallurgy. The discovery that copper alone is effective in improving the machinability of steel is believed to constitute an important advance in the technology of such steels, particularly since along with achieving improvement in machinability, desirable improvements in physical and mechanical properties are also secured. Such improvements have not been obtainable with elements previously added to modify the chemistry of steel to improve machinability.

Little, if any, improvement in machinability is secured when copper is present in the plain carbon or alloy steel in amounts less than 0.06 percent by weight. Best results are secured and a marked improvement in machinability as well as other physical and mechanical properties, such as impact strength, corrosion resistance, and tensile strength are secured when copper is present in the steel in amounts within the range of 0.15 to 0.30 percent by weight. To the present, improvements in the machinability of the steel have been secured by the use of copper in amounts up to 0.60 percent by weight, but it will be understood that the improvements in machinability can be secured by the use of copper in greater amounts.

Improvements in machinability of steel by the use of copper are noticeable with low carbon steel (less than 0.25 percent carbon) as well as with medium carbon steel (0.25 to 0.50 percent carbon) and high carbon steels (above 0.5 percent carbon). The general effect, for example, is illustrated in Table I in which a steel containing approximately 0.45 percent carbon was tested in a screw machine. For comparison, a steel of substantially the same composition was employed except for the presence of copper in one and the absence of copper in the other. A measure of the relative machinability was obtained by measuring the wear on the tools after 90 of the parts being machined had been cut under substantially identical conditions.

Table I

| Steel  | Chemistry |      |      |     |     |     | Machinability<br>(measured by tool<br>wear in inches) |                         |           |
|--------|-----------|------|------|-----|-----|-----|-------------------------------------------------------|-------------------------|-----------|
|        | C         | Mn   | S    | Ni  | Cr  | Cu  | 1/8" Turn-<br>ing Tool                                | 1/16" Turn-<br>ing Tool | Form Tool |
| 1----- | 0.43      | 1.44 | 0.25 | .05 | .05 | .05 | .012                                                  | .025                    | .013      |
| 2----- | 0.46      | 1.48 | 0.27 | .05 | .05 | .14 | .010                                                  | .009                    | .008      |

In the test described in Table I, parts were machined in a cycle time of 60 seconds, using a surface speed of 125 feet per minute and tool wear was measured after 90 pieces had been cut. The difference in Tool Wear is an indication of the difference in machinability of the two steels.

It will be apparent from the data secured that the steel containing copper showed approximately 17 percent better

wear on the  $\frac{3}{8}$  inch turning tool; 64 percent better tool wear on the  $\frac{1}{2}$  inch turning tool, and 38 percent better tool wear on the form tool.

The inventive concepts can be further illustrated by the effects of copper on the machinability of a low carbon steel (Table II).

Table II

| Steel | C    | Mn   | P    | S    | Si   | Ni    | Cr    | Cu   | Machinability <sup>1</sup> |
|-------|------|------|------|------|------|-------|-------|------|----------------------------|
| 1     | 0.17 | 0.69 | 0.03 | 0.03 | 0.05 | ----- | ----- | 0.04 | 74                         |
| 2     | 0.18 | 0.70 | 0.03 | 0.03 | 0.04 | ----- | ----- | 0.12 | 86                         |

<sup>1</sup> This is a comparative machinability reading obtained by controlled machining on a constant pressure lathe in a standard test. (Transactions of the ASME for July 1949 Constant-Pressure Lathe Test for Measuring the Machinability of Free-Cutting Steels, by F. W. Boulger, H. L. Shaw, and H. E. Johnson.)

In the past it has been recognized that residual metals such as nickel and chromium have caused marked depreciation in the machinability of steels even when present in small amounts. Contrary to the accepted limitations, it has been found that the deleterious effects of the residual metals on machinability of steels is reduced by the use of copper in accordance with the practice of this invention. While it is preferred to make use of a steel in which such residual metals are not present since copper is capable then of maximum use, it has been found that the presence of residual metals does not destroy the machinability characteristic of the steel in the presence of copper even though less improvement is secured by copper, nevertheless a steel containing copper in combination with the residual metals provides for better machinability than the same steel without copper or without the residual metals and copper.

Table III

| O   | Mn   | S    | Ni  | Cr  | Cu  | Cycle Time, Sec. | Surface Speed Per Min. | No. of Pieces Cut | Change in Size               |           |
|-----|------|------|-----|-----|-----|------------------|------------------------|-------------------|------------------------------|-----------|
|     |      |      |     |     |     |                  |                        |                   | $\frac{3}{8}$ " Turning Tool | Form Tool |
| .43 | 1.44 | .247 | .05 | .05 | .05 | 60               | 125                    | 90                | .004                         | .002      |
| .44 | 1.43 | .310 | .02 | .02 | .08 | 60               | 125                    | 90                | .001                         | .000      |
| .46 | 1.53 | .258 | .18 | .18 | .19 | 60               | 125                    | 90                | .002                         | .001      |

It will be apparent from the above table that the tool wear of medium carbon steels of similar composition are

in the machinability available from the copper is thusly effected.

It has been found that the improvement in machinability available from the use of copper in plain carbon steels and alloy steels can be extended by the addition of other elements with the copper, such for example as phosphorus, sulphur and nitrogen. To some extent these other elements have been used before because of their beneficial effects on machinability but the improvement

which is secured in a system which makes use both of copper and sulphur together in plain carbon and alloy steels exceeds that which might be expected by way of aggregation to the extent that improvement in machinability is indicative more of a synergistic effect between these materials in steel. These unexpected results are secured when sulphur is present in amounts ranging from 0.01 to 1.0 percent by weight in the steel and when the copper is present in an amount within the range of 0.06 to 0.6 percent by weight of the steel.

When phosphorus is present, the best results are secured when the concentration of phosphorus is within the range of 0.01 to 0.2 percent by weight, and the copper is present within an amount ranging from 0.06 to 0.6 percent by weight, and sulphur, when present, is present in an amount less than 1.0 percent by weight. Nitrogen in amounts greater than 0.001 percent by weight also improves the machinability of steel when present with copper alone or in a system which includes copper and one or more other elements, such as sulphur, phosphorus and nitrogen.

The following steels of the non-austenitic type are representative of the chemistries of steel or other iron base alloys embodying the features of this invention having improved machinability. In the examples the amounts

| C       | Cu      | Mn        | P       | Si      | Ni    | Mo      | Cr       | S       | N     |
|---------|---------|-----------|---------|---------|-------|---------|----------|---------|-------|
| .40-.48 | .06-.60 | 1.35-1.65 | <.04    | .17-.22 | <.05  | -----   | <.05     | .15-0.5 | ----- |
| .40-.48 | .06-.60 | 1.35-1.65 | <.04    | .17-.22 | <.05  | -----   | <.05     | .15-0.5 | ----- |
| .40-.48 | .06-.60 | 1.35-1.65 | .01-.20 | .17-.22 | <.05  | -----   | <.05     | .01-1.0 | ----- |
| .40-.48 | .06-.60 | 1.35-1.65 | .01-.20 | .17-.22 | <.05  | -----   | <.05     | .01-1.0 | ----- |
| .40-.48 | .06-.60 | 1.35-1.65 | .01-.20 | .17-.22 | <.05  | -----   | <.05     | .01-1.0 | >.001 |
| .40-.48 | .06-.60 | 1.35-1.65 | .01-.20 | .17-.22 | <.05  | -----   | <.05     | .01-1.0 | >.001 |
| .15-.23 | .06-.60 | 1.35-1.65 | <.04    | .17-.22 | <.05  | -----   | <.05     | .15-0.5 | ----- |
| .15-.23 | .06-.60 | 1.35-1.65 | <.04    | .17-.22 | <.05  | -----   | <.05     | .15-0.5 | ----- |
| .15-.23 | .06-.60 | 1.35-1.65 | .01-.20 | .17-.22 | <.05  | -----   | <.05     | .01-1.0 | ----- |
| .15-.23 | .06-.60 | 1.35-1.65 | .01-.20 | .17-.22 | <.05  | -----   | <.05     | .01-1.0 | ----- |
| .15-.23 | .06-.60 | 1.35-1.65 | .01-.20 | .17-.22 | <.05  | -----   | <.05     | .01-1.0 | ----- |
| .15-.23 | .06-.60 | 1.35-1.65 | .01-.20 | .17-.22 | <.05  | -----   | <.05     | .01-1.0 | ----- |
| .33-.41 | .06-.60 | .75-1.0   | <.04    | .20-.35 | ----- | .15-.25 | .80-1.10 | <.04    | ----- |

improved as much as 400 percent by the addition of copper and that the presence of nickel and chromium reduces the improvement secured by the presence of copper, yet the copper present with such residual elements provides for an improvement in machinability over and above the alloy without copper. In accordance with the information which has been developed to the present, the residual metals can be present in amounts totaling 0.25 percent by weight of the steel with a maximum of 0.05 percent by weight of any one element before improvement

in the manufacture of steel and other iron base alloys, copper may be introduced into the metal when in the furnace, ladle or mold, in the form of elemental copper, copper oxygen sulphide, copper sulphide or as copper sulphate or as a master metal containing copper, such as an iron-copper-sulphur alloy. It is an important concept of this invention that by the addition of copper in the forms described, normal operating procedures may be employed in the metallurgical processes for preparation of the steel. Recoveries of copper are essentially 100

percent and such additions to incorporate copper can be made without hazards and without requiring precautionary steps to be taken for the safety of personnel or equipment.

An important concept of this invention resides in the further discovery that the machinability of steel, for example as measured by the constant pressure lathe test previously described, especially steels having copper present in the amounts described, show unexpectedly large improvements in machinability when "cold worked." As used herein, the term "cold working" is meant to include deformation of the steel, as by cold drawing or rolling at room temperature or at elevated temperatures, such as described in copending applications Ser. No. 293,431, now abandoned, Ser. No. 293,432, now abandoned, and Ser. No. 293,433, now abandoned. The most striking effects by way of improved machinability by cold working become apparent with steels containing 0.50 carbon or less. Particularly outstanding results are secured with steels having 0.15 to 0.35 percent carbon. To the present, such improvements in machinability are maximized by cold working the steel for reduction in excess of 10 percent in cross sectional area and generally with reductions of between 20-50 percent depending upon the chemistry of the metal, the size of the raw material being cold worked, and in the case of drawing at elevated temperatures, the temperature of drawing.

The unexpected improvement in machinability of steel by cold working is illustrated by the following table which compares a steel having copper with the steel of the same composition except for copper. The two steels were reduced by cold drawing bars at room temperature, cold drawing bars which are at room temperature followed by strain relieving at high temperature, and cold drawing bars which are at an elevated temperature. Raw material for the test was hot rolled bar stock 1½ inches in diameter.

Table IV

|                                                            | Composition A | Composition B |
|------------------------------------------------------------|---------------|---------------|
| Carbon                                                     | .142          | .142          |
| Manganese                                                  | 1.22          | 1.11          |
| Phosphorus                                                 | 0.018         | 0.017         |
| Sulphur                                                    | 0.274         | 0.298         |
| Silicon                                                    | 0.05          | 0.03          |
| Chromium                                                   |               |               |
| Nickel                                                     |               |               |
| Molybdenum                                                 |               |               |
| Aluminum                                                   | 0.023         | 0.023         |
| Copper                                                     | 0.01          | 0.12          |
| Machinability Index: <sup>1</sup>                          |               |               |
| 10% draft at room temperature followed by strain relieving | 110           | 155           |
| 10% draft at elevated temperature                          | 111           | 162           |
| 15% draft at room temperature                              | 107           | 143           |
| 21% draft at room temperature                              | 106           | 155           |

<sup>1</sup> See footnote Table II.

It will be apparent from the data set forth in the above table that the machinability of steels containing copper within the amounts described is unexpectedly greatly improved by cold reductions, for example as by more than a 10 percent reduction in cross sectional area on a 1 inch bar, as compared to the machinability characteristics of steel having less than the described amounts of copper. When steel is drawn at about room temperature to achieve the desired reduction, strain relieving by heat treatment at a temperature above 550° F. but below the lower critical temperature and preferably within the range of 550-950° F. may be desirable. With steels having from 0.2 to 0.4 percent carbon, maximum improvement in machinability is secured by taking heavy drafts which may be followed by strain relieving, especially when copper is present in such steels alone or in a system with sulphur and with less than 0.15 residual metals composed of nickel, chromium and molybdenum. When working is achieved by drawing at elevated tem-

peratures as described in the aforementioned copending applications, subsequent strain relieving steps by heat treatment become unnecessary.

While cold working has been found to be desirable to improve the machining characteristics of steel, the combination of cold working steels of the type heretofore described containing copper alone or containing copper in a system with sulphur, and/or nitrogen, offers still further possibilities for providing high levels of machinability together with improved strength, resistance to corrosion, toughness, wear and other mechanical and physical properties without introducing limitations in the processing characteristics of the steel.

The unexpected improvements in machinability secured by metal working is not fully understood. It has been found that steels, particularly those containing carbon in the range of from 10-30 percent, can appreciably be benefited by heavy cold working. These beneficial effects with respect to machinability are enhanced when the steel contains copper alone or in the presence of phosphorus, sulphur, and/or nitrogen. Whatever the reason, the machinability of steels and iron base alloys, as determined by the energy required for metal separation and by reduction in wear of the turning and forming tools has been found greatly to be improved by modification in the chemistry of the steel to include copper as an essential component thereof, and further by working of the steel as by cold drawing to secure heavy drafts. Such improvements in machinability have been instrumental in accelerating output of steel products by enabling processing with heavy feeds and higher speeds to increase the production rate while at the same time reducing the time required for replacement and repair of tools and parts. In addition to increased output at reduced costs, the presence of copper to improve machinability has also provided improvements in other physical and mechanical properties as previously pointed out.

Though not equivalent, it is suggested that improvement in machinability of such iron base alloys and steel can be obtained by the addition of cobalt, zinc, cadmium, mercury, or tin. The chemical combination of these other elements in steel or other iron base alloys appears to correspond more with that observed for copper as compared to that from lead. The amounts required of these other elements are somewhat similar to that for copper with variations depending upon the solubility of the element in the iron or steel base alloy and the particular chemistry of the steel.

It will be understood that changes may be made in the details of formulation, methods of incorporation and processing of the various steels prepared in a manner to provide the characteristics of this invention without departing from the spirit of the invention, especially as defined in the following claims.

I claim:

1. The metallurgical process for improving the machinability of steel comprising the steps of advancing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, and less than 0.25 percent by weight residual metals selected from the group consisting of nickel, chromium, vanadium and molybdenum, with a maximum of 0.05 percent by weight of any one residual metal, and subsequently machining the steel to produce parts.

2. The metallurgical process for improving the machinability of steel comprising the steps of advancing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, and less than 0.25

percent by weight residual metals selected from the group consisting of nickel, chromium, vanadium and molybdenum, with a maximum of 0.05 percent by weight of any one, strain relieving the steel, and subsequently machining the steel to produce parts.

3. The metallurgical process for improving the machinability of steel comprising the steps of drawing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, and less than 0.25 percent by weight residual metals selected from the group consisting of nickel, chromium, vanadium and molybdenum, with a maximum of about 0.05 percent by weight of any one residual metal, and subsequently machining the steel to produce parts.

4. The metallurgical process for improving the machinability of steel comprising the steps of drawing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, and less than 0.25 percent by weight residual metals selected from the group consisting of nickel, chromium, vanadium and molybdenum, with a maximum of about 0.05 percent by weight of any one residual metal, strain relieving the steel, and subsequently machining the steel to produce parts.

5. The metallurgical process for improving the machinability of steel comprising the steps of extruding the steel through a die to effect reduction in cross-sectional area wherein the steel is a free machining steel of the non-austenitic type having copper and sulphur present as essential elements in the range of 0.15 to 0.30 percent by weight copper and 0.04 to 0.50 percent by weight sulphur, and less than 0.25 percent by weight residual metals selected from the group consisting of nickel, chromium, vanadium and molybdenum, with a maximum of 0.05 percent by weight of any one residual metal, and subsequently machining the steel to form parts.

6. The metallurgical process for improving the machinability of steel comprising the steps of advancing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, 0.01 to 0.20 percent by weight phosphorus, and less than 0.25 percent by weight residual metals selected from the group consisting of nickel, chromium, vanadium and molybdenum, with a maximum of 0.05 percent by weight of any one, and subsequently machining the steel to form parts.

7. The metallurgical process for improving the machinability of steel comprising the steps of advancing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, 0.01 to 0.20 percent by weight phosphorus, more than 0.001 percent by weight nitrogen, and less than 0.25 percent by weight residual metals selected from the group consisting of nickel, chromium, vanadium and molybdenum, with a maximum of 0.05 percent by weight of any one, and subsequently machining the steel to form parts.

8. The metallurgical process for improving the machinability of steel comprising the steps of advancing the steel through a die to effect reduction in cross-sectional area wherein the steel is a free machining steel of the non-austenitic type having copper present as an essential element in the range of 0.15 to 0.30 percent by weight, 0.04 to 0.50 percent by weight sulphur, 0.01 to 0.20 percent by weight phosphorus, more than 0.001 percent by

weight nitrogen, and less than 0.25 percent by weight residual metals selected from the group consisting of nickel, chromium, vanadium and molybdenum, with a maximum of 0.05 percent by weight of any one, strain 5 relieving the steel, and subsequently machining the steel to form parts.

9. The metallurgical process for improving the machinability of steel comprising the steps of advancing the steel through a die to effect reduction in cross-sectional area  
10 wherein the steel is a low carbon free machining steel of the non-austenitic type having up to 0.5 percent by weight carbon, copper present as an essential element in an amount within the range of 0.15 to 0.30 percent by weight, 0.04 to 0.50 percent by weight sulphur, and less  
15 than 0.25 percent by weight residual metals selected from the group consisting of nickel, chromium, vanadium and molybdenum with a maximum of 0.05 percent by weight of any one, and subsequently machining the steel to form parts.

parts.

20 10. The metallurgical process for improving the machinability of steel comprising the steps of heating the steel to a temperature within the range of 450° F. to the lower critical temperature for the steel composition, advancing the heated steel through a die to effect reduction in cross-sectional area while the steel is at a temperature within the range of 450° F. to the lower critical temperature for the steel composition and wherein the steel is a free machining steel of the non-austenitic type having copper present as an essential element in an amount within the range of 0.15 to 0.30 percent by weight, 0.04 to 0.50 percent by weight sulphur, and less than 0.25 percent by weight residual metals selected from the group consisting of nickel, chromium, vanadium and molybdenum with a maximum of about 0.05 percent by weight of any one, and subsequently machining the steel to form parts.

25

30

35

parts.

40 11. The metallurgical process for improving the machinability of steel comprising the steps of heating the steel to a temperature within the range of 450° F. to the lower critical temperature for the steel composition, advancing the heated steel through a die to effect reduction in cross-sectional area while the steel is at a temperature within the range of 450° F. to the lower critical temperature for the steel composition and wherein the steel is a free machining steel of the non-austenitic type having copper present as an essential element in an amount within the range of 0.15 to 0.30 percent by weight, 0.04 to 0.50 percent by weight sulphur, and less than 0.25 percent by weight residual metals selected from the group consisting of nickel, chromium, vanadium and molybdenum with a maximum of 0.05 percent by weight of any one, strain relieving the steel, and subsequently machining the steel to form parts.

45

50

12. The metallurgical process for improving the machinability of steel comprising the steps of advancing the steel through a draw die to effect reduction in cross-sectional area while the steel is at a temperature within the range of 450° F. to the lower critical temperature for the steel composition and wherein the steel is a free machining steel of the non-austenitic type having up to 0.50 percent by weight carbon, 0.15 to 0.30 percent by weight copper, 0.04 to 0.50 percent by weight sulphur, 0.1 to 0.20 percent by weight phosphorus, more than 0.001 percent by weight nitrogen, and less than 0.25 percent by weight residual metals selected from the group consisting of nickel, chromium, vanadium and molybdenum with a maximum of 0.05 percent by weight of any one, and subsequently machining the steel to form parts.

13. The metallurgical process for improving the machinability of steel comprising the steps of advancing the steel through a draw die to effect reduction in cross-sectional area while the steel is at a temperature within the range of 450° F. to the lower critical temperature for the steel composition and wherein the steel is a free machin-

ing steel of the non-austenitic type having up to 0.50 percent by weight carbon, 0.15 to 0.30 percent by weight copper, 0.04 to 0.50 percent by weight sulphur, 0.01 to 0.20 percent by weight phosphorus, more than 0.001 percent by weight nitrogen, and less than 0.25 percent by weight residual metals selected from the group consisting of nickel, chromium, vanadium and molybdenum with a maximum of 0.05 percent by weight of any one, heating to an elevated temperature to strain relieve the steel, and subsequently machining the steel to form parts.

5

**References Cited in the file of this patent**

**UNITED STATES PATENTS**

1,957,427 Buckholtz ----- May 8, 1934

|           |                |               |
|-----------|----------------|---------------|
| 2,281,132 | Young -----    | Apr. 28, 1942 |
| 2,320,040 | Landis -----   | May 25, 1943  |
| 2,400,866 | Kronwall ----- | May 21, 1946  |

**FOREIGN PATENTS**

|         |                   |               |
|---------|-------------------|---------------|
| 212,681 | Switzerland ----- | Mar. 17, 1941 |
| 677,967 | France -----      | Dec. 19, 1949 |

**OTHER REFERENCES**

10 "Metals Handbook," 1948 ed., pp. 309, 310, 369, 370, 537.

"Open Hearth Proceedings," pub. by AIMME, vol. 38, pp. 130-133.